

Dec. 9, 1924.

1,518,337

J. F. MAKOWSKI

PLASTER LATH

Filed March 4, 1924



INVENTOR.

*John F. Makowski*

BY

*Percy J. Webster*

ATTORNEY

## UNITED STATES PATENT OFFICE.

JOHN F. MAKOWSKI, OF STOCKTON, CALIFORNIA, ASSIGNOR TO CALIFORNIA CEDAR PRODUCTS COMPANY, OF STOCKTON, CALIFORNIA, A CORPORATION.

## PLASTER LATH.

Application filed March 4, 1924. Serial No. 696,768.

To all whom it may concern:

Be it known that I, JOHN F. MAKOWSKI, a citizen of the United States, residing at Stockton, county of San Joaquin, State of California, have invented certain new and useful Improvements in Plaster Laths; and I do declare the following to be a full, clear, and exact description of the same, reference being had to the accompanying drawings, 10 and to the characters of reference marked thereon, which form a part of this application.

This invention relates to the building art and particularly to wall construction. 15 The object of the invention is to produce a type of plaster lath similar to that described in detail in my allowed application for patent, Serial No. 608,595, in which asphalt can be used as the water proof element for the surfacing of the plaster board to which the finely divided mineral fragments are adhered. My aim in the invention is to mix with the asphaltum a hardening element so that when subjected to heat 25 it will not readily soften.

The figure of the drawings is a cross sectional view of a piece of my improved lath.

In the drawing the numeral 1 designates 30 the base board of the lath, preferably plaster board, 2 designates the adhesive surface lamination to which the mineral fragments 3 are adhered.

In the manufacture of the lath the material for the lamination 3 is made up of an 35 emulsion of asphalt and silicate of soda in the preferred proportions of thirty parts asphalt to seventy parts of silicate of soda.

This emulsion is spread over the base

board 1 to the proper thickness and the mineral fragments sprinkled and imbedded thereon by any suitable means. 40

The lath is then allowed to dry, the silicate of soda hardening and setting the asphalt so as to prevent its readily softening 45 under heat.

In the completed board the asphalt lamination forms a water proofing surface between the gravel and the base board as is 50 of importance in a board to render it a commercial success.

While I have herein set forth the preferred elements of the improved board, still in practice I may make such deviations therefrom as may fall within the scope of the 55 invention as defined by the appended claims.

Having thus described my invention what I claim as new and useful and desire to secure by Letters Patent is:

1. Plaster lath comprising a base, a surface lamination thereon consisting of asphalt and a hardening element, and finely divided mineral fragments adhered to such lamination. 60

2. Plaster lath comprising a base, a surface lamination thereon consisting initially of an emulsion of asphalt and silicate of soda, and finely divided mineral fragments adhered to such lamination. 65

3. Plaster lath comprising a base, a surface lamination thereon consisting initially of an emulsion of asphalt and silicate of soda in the proportions of thirty parts asphalt to seventy parts silicate of soda, and finely divided mineral fragments adhered to 75 such lamination.

In testimony whereof I affix my signature.  
JOHN F. MAKOWSKI.